

## UNITED STATES PATENT OFFICE

2,420,902

## LUBRICATING COMPOSITION

Arnold J. Morway, Clark Township, Union County, and John C. Zimmer, Union, N. J., assignors to Standard Oil Development Company, a corporation of Delaware

No Drawing. Application December 8, 1943,  
Serial No. 513,475

7 Claims. (CL. 252—36)

1

The present invention relates to lubricating compositions and more particularly to lubricating compositions especially adaptable for the lubrication of the mechanical parts of under-water craft.

Mechanical parts and mechanisms which are designed to operate in contact with water either intermittently or continuously as when completely submerged and depending upon some material or substance other than water for lubrication present a very troublesome lubricating problem. Situations of this nature arise in connection with under-water pumps where the complete mechanism remains submerged or is intermittently in contact with water, and in the case of under-water craft operation the need for special type lubricants becomes acute. The external mechanisms with which a submarine is equipped, such as conning tower hatch hinges, torpedo tube ports, periscope elevating mechanism and more recently gun carriages as well as various internal mechanisms must be lubricated. A lubricant for any of these purposes should be first water-insoluble or substantially water-insoluble. Secondly, such a lubricant should have a density greater than that of sea water. Water-insoluble lubricants have been proposed for use in contact with water, but their use has not been completely satisfactory, particularly in connection with submarine operation. Prior lubricants, being lighter than water, tend to be washed away and float to the surface. Also the lubricants used within the submersible tend to find their way into the bilge water, due to leaks around bearings and other causes, where they float. When the bilge water is pumped out these waste and used lubricants float to the surface causing oil slicks and wakes. These slicks and wakes are an almost certain indication of the presence of submersibles, are readily seen by observers on surface or airborne craft, thereby making the detection of under-water craft relatively simple.

An object of the present invention is the production of a lubricating composition which is insoluble in water. Another object is the provision of a lubricating composition having a density greater than sea water. Another object is to produce a lubricant which will be non-inflammable, and thus usable in applications such as lubrication of equipment manufacturing munitions, explosives, incendiaries or in any application of lubricants where inflammable material which might be ignited by a spark of electrical, mechanical or chemical origin would be a hazard. These and other objects will be apparent to those skilled in the art upon reading the following description.

It has now been discovered that lubricants suitable for under-water and non-inflammable service can be made by employing a water-insoluble soap together with a halogenated aromatic

2

hydrocarbon in which the halogen is substituted in the aromatic ring nucleus. Such aromatic hydrocarbons may be represented by benzene, isopropyl benzene, naphthalene, diphenyl, triphenyl, toluene, xylene and homologous derivatives thereof, and the halogenated products in general by the empirical formula  $(\text{Hal}_n \text{ Arom R})_m \text{ H}_o$ , where Hal represents one of the halogens, chlorine, fluorine, bromine and iodine; Arom represents the benzene or naphthalene nucleus, R is hydrogen or an alkyl radical such as methyl, ethyl, propyl, isopropyl, etc., n and o are integers from 1-14 and m is an integer from 1-3. The preferred halogenated aromatic hydrocarbons are solids or oily liquids at ordinary temperatures having a density greater than 1.04. These halogenated aromatic hydrocarbons can be produced through the direct halogenation of the corresponding hydrocarbon and by other known means and are relatively stable to hydrolysis. It is further preferred to use those halogenated aromatic hydrocarbons containing from 20-60% of halogen on a weight basis. Solid halogenated aromatic hydrocarbons may be dissolved in liquid halogenated hydrocarbons to obtain the required or desired density and fluidity. Compounds containing halogen substituted in an aliphatic or alkyl radical should not be used for the purposes of this invention for the reason that compounds of this nature readily hydrolyze, yielding halogen acids. Specific examples of those halogenated aromatic hydrocarbons falling within the purview of the present invention are chloro-, bromo-, or iodobenzene; chloro-, bromo-, iodo- or fluorodiphenyl; methyl chlorobenzene, methyl dichlorobenzene; isopropyl trichlorobenzene, dimethylchlorobenzene, chloronaphthalene, etc. Unless specific steps are taken to purify the product, halogenation of aromatic hydrocarbons results in a mixture of halogenated products, and for the purposes of the present invention, such a mixture need not be purified or further modified if it is of the proper density. It is intended that the lubricants of the present invention shall contain from 70-95% of halogenated aromatic hydrocarbons.

For the formation of the soaps utilized in the production of the grease composition of this invention, any soap stock, such as saturated or unsaturated fats of either vegetable or animal origin, such as stearin or cotton seed oil or the saturated or unsaturated fatty acid derived therefrom such as stearic acid or oleic acid may be used, although it is preferred to use the saturated acids derived from hydrogenated fish oil. The soaps derived from the soap stocks must be water-insoluble, and for this purpose, neutralizing or saponifying agents are used, such as lithium, calcium, barium, strontium, aluminum, zinc or lead, which react with fatty acids to form water-insoluble soaps. The preferred composi-

tions also include a buffering agent, such as aluminum stearate for stabilizing the hydrogen-ion concentration, and an oxidation inhibitor such as zinc naphthenate, the zinc salt of a mono-carboxylic acid having more than six carbon atoms, a zinc phenate or a zinc salt of an alkylated phenol, phenol sulfide or thiophosphate. The amount of soap in the composition will vary somewhat ranging generally between 5 and 30% by weight, according to the consistency desired in the final product. Compositions containing from 5-10% of soap are semi-fluid products, while if 12 to 30% or more of soap is present, greases of firm structure increasing in consistency with rising soap content are obtained. The amount of buffer and oxidation inhibitor used will each range from about 0.1-1% by weight. The compositions herein described have no flash point and the spontaneous ignition point is above 1000° F.

In most instances, any of the methods customarily employed in the compounding of greases may be used in the production of the compositions of this invention, however, some halogenated hydrocarbons readily volatilize on heating, in which case the soaps may be produced separately and then mixed with the halogenated hydrocarbon by heat and agitation. Where the soap is made separately the soap stock is first melted and then an aqueous solution or suspension of the alkaline material is added and the mixture is heated and stirred until the reaction is complete, after which the temperature is raised to boil off the water. The remainder of the materials may then be added and the temperature raised until a fluid grease is obtained which is generally in the range from 250°-360° F. These compositions made in accordance with the foregoing description have been found to possess very marked characteristics in that they will not float in water and are water-insoluble.

The following examples will serve to illustrate the principles of the present invention.

#### Example 1

|                                                     | Per cent |
|-----------------------------------------------------|----------|
| Hydrogenated fish oil acid                          | 13.00    |
| Lithium hydroxide monohydrate                       | 2.05     |
| Zinc naphthenate                                    | 0.50     |
| Aluminum stearate                                   | 0.50     |
| Chlorinated diphenyl containing 48% Cl <sub>2</sub> | 83.95    |

The hydrogenated fish oil acid and about 20% of the chlorinated diphenyl were charged to a kettle equipped with a stirrer, heating was started and when all the acid had melted the lithium hydroxide dissolved in as small an amount of boiling water as possible was added. After the soap was formed, heating was continued to around 200° F. until most of the water was removed. Approximately 60% of the remainder of the chlorinated diphenyl was then added and the temperature raised to 300° F. A sample was then taken for alkalinity determination which should be from 0.1-0.2 figured as NaOH and the alkalinity of the batch was adjusted accordingly. The aluminum stearate, dispersed in the balance of the chlorinated diphenyl, was then added along with the zinc naphthenate to the kettle and the temperature was raised until the grease became fluid at about 360° F. Stirring and heating were then discontinued and the grease allowed to cool. After cooling the grease was

worked to a smooth paste in the kettle and then filtered.

|   |                                   |     |
|---|-----------------------------------|-----|
| 5 | A. S. T. M. penetration, unworked | 266 |
|   | A. S. T. M. penetration, worked   | 303 |
|   | Dropping point, °F                | 356 |

#### Example 2

|                                                     | Per cent |
|-----------------------------------------------------|----------|
| Hydrogenated fish oil acid                          | 13.00    |
| 10 Lithium hydroxide monohydrate                    | 2.05     |
| Aluminum stearate                                   | 0.50     |
| Zinc naphthenate                                    | 0.50     |
| Tri - chlor - benzene                               | 25.185   |
| Chlorinated diphenyl containing 48% Cl <sub>2</sub> | 58.765   |

15 In compounding the composition of the example the hydrogenated fish oil acid and chlorinated diphenyl were heated together as described in Example 1, reacted with lithium hydroxide, heated to remove water after which the balance of the chlorinated diphenyl was added, the temperature raised to 300° F. and the batch adjusted for alkalinity. The aluminum stearate dispersed in the tri-chlor-benzene, together with the zinc naphthenate was then added to the kettle and the temperature was raised to the melting point of the grease. Stirring and heating were then discontinued and the grease allowed to cool after which the grease was worked to a smooth paste and filtered as described in Example 1. By operating in this manner, maximum control of the vapors of tri-chlor-benzene was obtained.

|    |                                   |     |
|----|-----------------------------------|-----|
| 35 | A. S. T. M. penetration, unworked | 300 |
|    | A. S. T. M. penetration, worked   | 305 |
|    | Dropping point, °F                | 352 |

What is claimed is:

1. A lubricating composition consisting of about 84% of an isomeric mixture of chlorinated diphenyl containing an average of 48% of chlorine, 15% lithium soap of hydrogenated fish oil acids, .5% aluminum stearate and .5% zinc naphthenate.

45 2. A lubricant comprising 5-30% of water-insoluble metal soap wherein the metal of said soap is selected from the group consisting of lithium, calcium, barium, and strontium, 70-95% of an isomeric mixture of chlorinated diphenyl of 48% average chlorine content on a weight 50 basis, from 0.1 to 1% of aluminum stearate and from 0.1 to 1% of zinc naphthenate, said lubricant having a density greater than that of sea water.

55 3. A lubricating composition according to claim 2 in which the water-insoluble soap is a calcium soap.

4. A lubricating composition according to claim 2 in which the water-insoluble soap is a barium soap.

60 5. A lubricant comprising 5-30% of a water-insoluble metal soap wherein the metal of said soap is selected from the group consisting of lithium, calcium, barium, and strontium, about 25% of a halogenated aromatic hydrocarbon with

65 a single benzene ring nucleus and approximately 60% of an isomeric mixture of chlorinated diphenyl of 48% average chlorine content on a weight basis, stabilized and buffered by 0.1 to 1% of aluminum stearate and 0.1 to 1% zinc naphthenate, the said lubricant having a density greater than that of sea water.

70 6. A lubricant comprising 5-30% of a water-insoluble metal soap wherein the metal of said soap is selected from the group consisting of lithium, calcium, barium, and strontium, about

25% of a chlorinated aromatic hydrocarbon with a single benzene ring nucleus and approximately 60% of an isomeric mixture of chlorinated diphenyl of 48% average chlorine content on a weight basis, stabilized and buffered by 0.1 to 1% of aluminum stearate and 0.1 to 1% of zinc naphthenate, said lubricant having a density greater than that of sea water.

7. A lubricant composition consisting of about 25% trichlorbenzene, 59% of an isomeric mixture of chlorinated diphenyl containing an average of 48% chlorine, 15% lithium soap of hydrogenated fish oil acids, .5% aluminum stearate and .5% zinc naphthenate.

ARNOLD J. MORWAY. 15  
JOHN C. ZIMMER.

#### REFERENCES CITED

The following references are of record in the file of this patent:

#### UNITED STATES PATENTS

| Number    | Name      | Date          |
|-----------|-----------|---------------|
| 2,079,783 | Wiezevich | May 11, 1937  |
| 2,127,497 | Webster   | Aug. 23, 1938 |

| Number    | Name             | Date           |
|-----------|------------------|----------------|
| 2,274,674 | Earle I          | Mar. 3, 1942   |
| 2,283,602 | Fiero            | May 19, 1942   |
| 2,293,052 | Earle II         | Aug. 18, 1942  |
| 2,330,238 | Prutton          | Sept. 28, 1943 |
| 2,332,825 | Zimmer et al.    | Oct. 26, 1943  |
| 2,354,171 | Morgan           | July 18, 1944  |
| 2,360,631 | Zimmer et al.    | Oct. 17, 1944  |
| 2,363,013 | Morway et al.    | Nov. 21, 1944  |
| 1,982,198 | Brunstrum et al. | Nov. 27, 1934  |
| 1,989,196 | Hilliker et al.  | Jan. 29, 1935  |
| 2,245,772 | Gothard et al.   | June 17, 1941  |
| 2,383,148 | Morgan et al.    | Aug. 21, 1945  |

#### OTHER REFERENCES

Penning, Physical Characteristics and Commercial Possibilities of Chlorinated Diphenyl, Article in Industrial and Engineering Chemistry, vol. 22, pp. 1180, 1181, and 1182, Nov. 1930, 260-74. Plasticizers and Resins, pub. by Monsanto Chemicals, revised May 1940, page 34. (Copy in Div. 50.)

The Arochlors, Application Data Bulletin No. P-115, pub. by Monsanto Chemical Co. of St. Louis, page 13. (Copy in Div. 64.)